

## 1

3,335,477

## PROCESS FOR CRIMPING DIFFICULTLY CRIMPABLE FIBERS

Harold Edward Arnold, Kinston, N.C., assignor to E. I. du Pont de Nemours and Company, Wilmington, Del., a corporation of Delaware  
No Drawing. Filed Apr. 20, 1965, Ser. No. 449,624  
6 Claims. (Cl. 28—72)

This invention relates to highly crimped, high-denier fibers and more particularly to a crimping process for increasing the frequency of crimp in high-denier fibers.

It is well-known to employ stuffing-box crimpers such as that described in U.S. Patent No. 2,311,174 to crinkle continuous filament fibers. The crinkled, or crimped fibers may then be employed as a bundle of continuous filaments or may be cut to staple length for processing on one of the known staple processing systems such as the cotton system, worsted system, garnetter, etc. to yield structures resembling those of natural fibers in bulk and tactility.

An object of this invention is to provide a process for the high frequency crimping of difficultly crimpable continuous filaments. Another object is to provide a process for crimping of high denier continuous filaments in a stuffing box to increase the crimp frequency. Other objects will appear hereinafter.

The objects of this invention are accomplished, in general, by a process for increasing the frequency of stuffing box crimp in difficultly crimpable continuous filaments which comprises admixing at least 10% by weight, based upon the total weight of continuous filaments, of easily crimpable continuous filaments with the difficultly crimpable continuous filaments to form a blend and thereafter crimping the blend in a stuffing box crimpler. The term "easily crimpable continuous filaments" is meant to define continuous filaments which, under the same operating conditions in a stuffing box crimpler, have a crimp frequency of at least 1.3 times that of the difficultly crimpable continuous filaments. In the preferred embodiment, the difficultly crimpable continuous filaments are continuous filaments having a denier per filament of at least 10; and the easily crimpable continuous filaments are continuous filaments which have a denier per filament of less than 10. More specifically, it is preferred to have a denier range of 30 to 50 for the difficultly crimpable continuous filaments and a denier range of 2 to 7 for the easily crimpable continuous filaments.

Although it is understood that the invention is not to be limited by theoretical considerations, it is hypothesized that Euler's formula for column collapse under a critical load applies to the step of crimping wherein the column (fiber bundle) is loaded to the point of collapse in a stuffing box. Thus,  $P = \pi EI/12$  states that the critical loading for collapse of a column (P) equals the product of a constant, the modulus of elasticity (E), and the moment of inertia (I) of the column divided by the square of its length. With a given polymeric composition comprising a range of fiber deniers and a crimpler of given geometry, the modulus of elasticity and column length remain relatively constant. It is apparent, therefore, that in this case the force required to bring about column collapse will vary as the moment of inertia of the filament, which is approximately proportional to the fourth power of the filament diameter (this is strictly true only in the special case where the filaments are circular in cross-section). Although column collapse as hereinbefore described presumes no lateral or bending forces which cooperate to encourage buckling, it is theorized that the easily crimpable continuous filaments do in fact impart a lateral force on neighboring more

## 2

difficultly crimpable continuous filaments to force an earlier collapse.

The following examples will serve to illustrate the invention, although they are not intended to be limitative. The examples were carried out using a stuffing box crimpler similar to that described in United States Patent No. 2,311,174, using conditions known to produce the maximum obtainable crimp frequency. The amount of closing force applied to the hinged gate which restricts egress of the crimped continuous filaments from the stuffing box was maintained at the maximum operable force. The force is determined by gradually increasing the gate pressure during normal operation until the crimpler "jams," i.e., until the feed rolls are no longer able to force additional tow of continuous filaments into the stuffing box. Once such force is determined, the maximum operable force is chosen to be just below the determined force. The determinations of the crimp frequency is made by straightening a length of crimped tow sufficiently to count the individual crimps, extending the tow under a load sufficient to remove all crimp and measuring the length of section in which the crimp was counted. Crimp frequency is reported in crimps per extended inch (c.p.i.) calculated by the following formula:

$$c.p.i. = \frac{\text{number of crimps counted}}{\text{length (inches) of section}}$$

## Example 1

Poly(ethylene terephthalate) of 0.5 intrinsic viscosity is melt spun to 104 filaments per spinneret substantially in accord with the process described in United States Patent No. 2,918,346. Approximately 200 such ends are combined to form a tow which is drawn 4.1 $\times$  (to 410% of its original length) by a process substantially as described in the aforementioned patent. The tow is dried and relaxed on a continuous-belt with circulating air maintained at 140° C.

The tow is then crimped in the stuffing box crimpler. The crimped tow has a denier-per-filament (d.p.f.) of 40 and a total denier of 840,000; tenacity is 2.7 g.p.d.; elongation at the break is 62%, and shrinkage at 196° C. in dry air is 7.1%. The resulting crimped tow has an average crimp frequency of 4.1 per inch (c.p.i.), with 20 determinations being made which ranged from 3.3—4.5 c.p.i.

## Example 2

Example 1 is repeated in all essential respects, except that the tow is blended with varying amounts of a 4.75 d.p.f. poly(ethylene terephthalate) tow, whose total denier is varied so as to result in the desired weight percent lower denier-per-filament fiber in the tow to be crimped. Blending of the two tows is accomplished in each case by arranging individual spun ends in an alternating pattern as they are fed to the drawing step, thereby accomplishing a reasonably uniform distribution of the low denier per filament product in the total.

Characterization of the crimp of the fiber blends is illustrated in Table I:

TABLE I

|                              | Percent 4.75 d.p.f. in tow |         |         |
|------------------------------|----------------------------|---------|---------|
|                              | 15                         | 30      | 50      |
| Tenacity (g.p.d.)            | 2.3                        | 3.4     | 2.9     |
| Elongation (percent)         | 70.3                       | 37.2    | 43.0    |
| Dry heat shrinkage (percent) | 7.2                        | 7.5     | 9.7     |
| Crimps per inch:             |                            |         |         |
| Average                      | 4.6                        | 5.4     | 6.0     |
| Ranges                       | 4.2—5.3                    | 4.9—6.5 | 5.2—7.5 |
| No. determinations           | 20                         | 20      | 20      |

As can be seen from Example 2, the average crimp frequency increases as increasing amounts of the smaller denier continuous filaments are added to the fiber blend. More significantly, however, is the fact that the minimum crimp frequency also increases. This illustrates that the higher denier filaments are being crimped to a higher frequency.

There is no upper limit with respect to the amount of the easily crimpable continuous filaments in the fiber blend. However, since the resulting crimped tow is not separated into its different component continuous filaments, a practical upper limit may be necessitated by specifications for the use to which the end product will be put. Additionally, the method by which the fiber blend is formed is not critical although it is preferred to have a uniform blend.

With regard to the stuffing box crimpler and its operation, it should be obvious that the particulars of the design are not critical. Also, the operating conditions of the crimpler may be varied as desired. The examples were run at the optimum conditions for producing maximum crimp frequency to illustrate the extent of the increase in the crimp frequency by utilizing the process of this invention. Depending upon the desired crimp frequency, the operating conditions may be varied.

The examples utilized continuous filaments prepared from polyethylene terephthalate, this being the best-known commercial polyester fiber. However, it should be obvious that other polyesters could be substituted with substantially equivalent results being had. Moreover, although it is preferred to utilize the same polymer to prepare both types of continuous filaments, there is no necessity that the same polymer be used. In fact, the characteristics desired in the crimped product might call for the use of two different polymers.

Additionally, the examples illustrate the practice of this invention by using easily crimpable continuous filaments of smaller denier to increase the crimp frequency of larger denier continuous filaments. It should be noted that other routes to easily crimpable continuous filaments could be advantageously utilized. For example, continuous filaments of intermediate denier per filament having a low modulus of elasticity or which change more rapidly in modulus when heated could be used. In this last instance, the heat could be supplied by contact with steam during the crimpling, for example.

The process of this invention provides a simple method for increasing crimp frequency in relatively high denier continuous filaments. This increased frequency finds particular utility when the crimped tow is used for stuffing materials. The higher frequency of the crimped tow gives improved ability to yield appreciably under small loads but to resist "bottoming" under large loads. This is an important characteristic of premium stuffings.

Since many different embodiments of the invention may be made without departing from the spirit and scope thereof, it is to be understood that the invention is not limited by the specific illustrations except to the extent defined in the following claims.

What is claimed is:

1. The process for increasing the frequency of stuffing box crimps in difficultly crimpable continuous filaments which comprises admixing at least 10% by weight, based upon the total weight of the continuous filaments of easily crimpable continuous filaments with said difficultly crimpable continuous filaments to form a blend and thereafter crimping said blend in a stuffing box crimpler whereby the crimping of the said easily crimpable continuous filaments imparts a lateral force on the said difficultly crimpable continuous filaments and thereby assists in the higher frequency crimping of the said difficultly crimpable continuous filaments.

2. The process for increasing the frequency of stuffing box crimps in difficultly crimpable continuous filaments which comprises admixing from about 10 to about 50% by weight, based upon the total weight of the continuous filaments of easily crimpable continuous filaments with said difficultly crimpable continuous filaments to form a blend and thereafter crimping said blend in a stuffing box crimpler whereby the crimping of the said easily crimpable continuous filaments imparts a lateral force on the said difficultly crimpable continuous filaments and thereby assists in the higher frequency crimping of the said difficultly crimpable continuous filaments.

15 3. The process for increasing the frequency of stuffing box crimps in first continuous filaments having a denier per filament of at least 10 which comprises admixing at least 10% by weight, based upon the total weight of continuous filaments of second continuous filaments having a denier per filament of less than 10 with said first continuous filaments to form a blend and thereafter crimping said blend in a stuffing box crimpler whereby the crimping of the said second continuous filaments imparts a lateral force on the said first continuous filaments and thereby assists in the higher frequency crimping of the first continuous filaments.

20 4. The process for increasing the frequency of stuffing box crimps in first continuous filaments having a denier per filament of at least 10 which comprises admixing from about 10 to about 50% by weight, based upon the total weight of continuous filaments of second continuous filaments having a denier per filament of less than 10 with said first continuous filaments to form a blend and thereafter crimping said blend in a stuffing box crimpler whereby the crimping of the said second continuous filaments imparts a lateral force on the said first continuous filaments and thereby assists in the higher frequency crimping of the first continuous filaments.

25 5. The process for increasing the frequency of stuffing box crimps in first continuous filaments having a denier per filament range of from about 30 to about 50 which comprises admixing at least 10% by weight, based upon the total weight of continuous filaments, of second continuous filaments having a denier per filament range of from about 2 to about 7 with said first continuous filaments to form a blend and thereafter crimping said blend in a stuffing box crimpler whereby the crimping of the said second continuous filaments imparts a lateral force on the said first continuous filaments and thereby assists in the higher frequency crimping of the first continuous filaments.

30 6. The process for increasing the frequency of stuffing box crimps in first continuous filaments having a denier per filament of about 40 which comprises admixing from about 10 to about 50% by weight, based upon the total weight of continuous filaments, of second continuous filaments having a denier per filament of about 4.75 with said first continuous filaments to form a blend and thereafter crimping said blend in a stuffing box crimpler whereby the crimping of the said second continuous filaments imparts a lateral force on the said first continuous filaments and thereby assists in the higher frequency crimping of the first continuous filaments.

35 7. The process for increasing the frequency of stuffing box crimps in first continuous filaments having a denier per filament of about 40 which comprises admixing from about 10 to about 50% by weight, based upon the total weight of continuous filaments, of second continuous filaments having a denier per filament of about 4.75 with said first continuous filaments to form a blend and thereafter crimping said blend in a stuffing box crimpler whereby the crimping of the said second continuous filaments imparts a lateral force on the said first continuous filaments and thereby assists in the higher frequency crimping of the first continuous filaments.

#### References Cited

##### UNITED STATES PATENTS

|    |           |         |                |        |
|----|-----------|---------|----------------|--------|
| 65 | 2,311,174 | 2/1943  | Hitt           | 28—72  |
|    | 3,009,310 | 11/1961 | Murchie et al. | 28—72  |
|    | 3,046,724 | 7/1962  | Ward           | 57—140 |

70 MERVIN STEIN, Primary Examiner.

L. K. RIMRODT, Examiner.